

Patented Apr. 14, 1953

2,635,052

3

## UNITED STATES PATENT OFFICE

2,635,052

## PRODUCTION OF CELLULAR CONCRETE BLOCKS

Peter Edward Starnes, Boreham Wood, England,  
assignor to John Laing & Son Limited, London,  
England, a British company

No Drawing. Application October 20, 1948, Serial No. 55,647. In Great Britain October 22, 1947

2 Claims. (Cl. 106—87)

1

The present invention relates to the production of cellular concrete for use in the manufacture of blocks, slabs, beams and the like and has for its object an improved composition and process of manufacture.

The manufacture of any light-weight cellular composition suitable for satisfactory use as a structural material in building presents two distinct problems.

(a) The problem of producing a paste or slurry of suitable siliceous substances capable of hardening into a strong, durable material possessing a minimum of microscopic capillaries and pores and exhibiting the smallest possible changes of dimensions on wetting and drying.

(b) The problem of inducing a uniform cellular, or foam-like, structure in the said paste or slurry, which will remain substantially unchanged during the subsequent processing and curing of the composition, so that a strong, light and relatively impermeable cellular material will result. In this connection it has been found that certain characteristics are desirable in the cellular structure, while others are equally undesirable. It is desirable that the structure shall consist of uniformly sized, spherical cells and that there shall be a minimum of interconnection between neighbouring cells. This is desirable, not only in order to attain the maximum strength for a given density, but also in order to restrict the circulation of air and water vapour throughout the composition, and hence to ensure the lowest possible thermal conductivity. It is undesirable that the cells should be distorted out of the spherical shape into ellipsoids so as to produce the appearance of an horizontally laminated structure when a vertical section of the material is viewed under the microscope. This fault, which is common in chemically expanded light-weight concrete results in a difference in the compressive strengths of the product when tested in two mutually perpendicular directions. It is also undesirable that large bubbles or voids be formed in the material either by the coalescence of small bubbles or by the accidental entrainment of air during the mixing or pouring of the composition.

In practice I have found that these two problems are actually inter-related in as much as attempts to reduce the movements on wetting and drying of the material by the incorporation of a quantity of coarser sand as described below will usually result in the formation of a more or less laminated structure, together with a variation in the size of the cells throughout the body of the composition when the latter is poured into moulds to form units suitable for use in building.

The present invention relates to both these problems. In the first place it has as an object an improved composition which when aerated

P/C  
ash  
— flyash or  
ground ash

sand  
alumina

calcium sulphate  
1,3-carboxymethyl cellulose  
ethyl methyl cellulose.

2

into a cellular structure and suitably cured as described herein, will form a light-weight cellular material of great strength and durability, which exhibits relatively small movements on wetting and drying. In the second place it has for an object an improvement to the known method of aerating such a composition by the production of a gas within the mass by the reaction of a finely divided metal and a weak solution of alkali whereby the uniformity of the cellular structure may be controlled and the tendency for the production of a laminated structure eliminated.

The restriction of the drying shrinkage and movement on wetting of any light-weight concrete composition within an acceptable limit is of primary importance if it is intended that the material should be suitable for exterior exposure in a normally constructed building. It is unfortunate in this respect that the circumstances which lead to the development of a high strength in a siliceous cement paste also tend to result in an increase in the movements on wetting and drying of the hardened product. This is particularly true in light-weight compositions of the type with which this invention is concerned. In this case it is essential in order to satisfy the requirements of strength and durability and at the same time retain a low density, that a fairly high proportion of cementing constituents be present in the hardened paste.

For this reason it is most important that the cementing constituents shall themselves be of a type exhibiting the minimum changes of dimensions on wetting and drying. It is known in the art that the admixture with a normal Portland cement of a small quantity of very finely ground trass or other natural pozzolana can result when cured at ordinary temperatures, in the formation of a hardened paste having lower shrinkage characteristics and a lower absorption than a paste of equivalent strength formed from the neat cement. This is attributed to the reduction in the uncombined lime content and the formation of a proportion of silicates of lower basicity such as mono-calcium silicate hydrate in the paste instead of the dicalcium silicate hydrate which is normally the principal compound formed during the hardening of a Portland cement paste. It is also known that curing a Portland cement paste at elevated temperatures in the presence of saturated steam will, provided the temperature is sufficiently high, result in a great reduction of the shrinkage and expansion of the hardened paste on drying and wetting. This is likewise to be attributed to the increased tendency for the formation of a crystalline silicate hydrate of low basicity. It is to be expected that a combination of both these methods, i. e. the incorporation of a proportion of finely divided active

silica and the use of high pressure steam curing would result in an even greater tendency for the formation of the monocalcium silicate hydrate, and this has been shown to be the case. By the choice of an appropriate source of finely divided active silica it has been found possible greatly to cheapen the cost of a suitable low shrinkage cementing material of great durability when compared with the cost of a normal Portland cement paste of equivalent strength and durability.

At the same time the rate of strength gain is much increased and hence the curing time reduced.

Further by the incorporation of a proportion of suitably graded sand with the cementing mixture I have found it possible to produce a hardened paste of great strength, durability and further improved shrinkage characteristics. This has been made possible by the discovery that certain chemical agents herein described are capable of exerting a strong stabilising influence on the cellular structure of the uncured paste so as to permit of the admixture of a proportion of coarser aggregate which would otherwise interfere with the development of a uniform structure and in particular result in the production of undesirable laminations.

It has previously been recorded that some samples of pulverised fuel ash exhibited slight pozzolanic activity when admixed with Portland cement in the preparation of ordinary dense concrete, and this is to be expected when the chemical nature and state of division of the material are considered.

I have studied the nature and reactivity of various samples of pulverised fuel ash, and have found that different samples vary greatly in their chemical reactivity. In general, it was possible to distinguish two main groups.

(a) Ash collected from the furnace gases by means of cyclone type separators. This type was always less reactive than type (b).

(b) Ash collected from the furnace gases by means of electrostatic precipitators. This type was always more reactive than type (a).

On microscopic examination of the samples it was found that all those of type (b) were characterised by containing a reasonable proportion of very fine particles (say less than 15 microns in diameter). Ashes of type (a) contained very much fewer particles smaller than about 15 microns in diameter. This fact affords a reasonable explanation of the difference observed in the reactivity of the two types of ash. Since the reaction is a surface reaction it is greatly favoured by the presence of a large number of ultra small particles having a very high specific surface. For example, below are given the specific surfaces in square centimetres per gramme of particles of different sizes having a specific gravity of 2.2 assuming all the particles to be smooth and spherical.

| Size of Particles | Surface Area of 1 grammme of Material |
|-------------------|---------------------------------------|
| 20 $\mu$          | 1,345                                 |
| 10 $\mu$          | 2,690                                 |
| 5 $\mu$           | 5,380                                 |
| 2 $\mu$           | 13,450                                |
| 1 $\mu$           | 26,900                                |
| 0.5 $\mu$         | 57,800                                |

From this it can be seen how important is the part played by the particles smaller than 15 $\mu$  and

particularly by ultra fine particles less than about 5 $\mu$  in diameter.

The problem of selection of a suitable ash is to some extent complicated by the fact that all samples of pulverised fuel ash contain a quantity of unburnt carbon, usually as irregular particles of coal or coke about 50-100 microns in size. If present in any considerable proportion this carbon exerts a deleterious effect upon the product.

- 10 This occurs in two ways. Firstly, the carbon may be regarded as an inactive adulterant which not only fails to contribute to the development of strength in the material, but may also by virtue of its own porosity and absorption increase the 15 porosity and movement on wetting and drying of the product. Secondly, it may so increase the quantity of water necessary to produce a suitable paste or slurry as further to detract from the quality of the product both as regards strength 20 and impermeability to water. Fortunately I have found that ashes with carbon contents in the range normally experienced (say 5-15%) can be used quite satisfactorily. It is wise however to select a source of ash so that the carbon content 25 does not exceed 10-12% if the maximum economy of cement is to be affected in the proportioning of the mix.

I have found that pulverised fuel ash when selected according to the above principles and 30 mixed together with Portland cement and a suitably graded siliceous sand and water in the correct proportions and aerated according to the method described below will on hardening give rise to a particularly strong and durable light-weight composition of low permeability. If the 35 full benefit of the composition is to be realised it is desirable to cure the material in high pressure steam at a temperature exceeding 175° C. This applies particularly when the product is desired to have a density less than 60-70 lbs./cu. ft. and when it is necessary to achieve the minimum changes in dimensions on wetting and drying.

With regard to the grading of the sand I have found that the use of stabilising agents described 40 below permits of a considerable latitude. The choice is of course influenced by the density which it is desired to achieve in the final product. In general the sand should have a high silica content, be clean, free from contamination 45 by clay or organic matter and have a grading in the range indicated below. A sand at the coarser end of the range is suitable for the denser products, while a sand of the finer type is suitable for the light-weight products and particularly for 50 products hardened in high pressure steam.

#### Range of suitable gradings

| B. S. Sieve No. | Percentage Passing |
|-----------------|--------------------|
| 60              |                    |
| 25.....         | 80-100             |
| 52.....         | 40-80              |
| 100.....        | 0-10               |

65 With regard to the improved method of aeration, it is known to induce a cellular structure in a paste or slurry of siliceous materials by the action of a dilute solution of alkali on a quantity 70 of finely divided metal incorporated in the slurry. I have found that although this method can be quite satisfactory in some cases when the solid matter present is all very fine (say less than B. S. S. No. 100) it often fails to produce the desired uniformity of structure when a propor-

tion of the coarser material is present. In particular two faults are liable to be developed in this case. The individual bubbles or cells become flattened into an ellipsoidal shape due to the tendency for the aerated slurry to settle slightly in the mould. Also it is common to find that the density of the material increases from the top to the bottom of the mould due to the compression of the lower bubbles. Both these faults become more serious as the depth of the mould is increased, and in fact set a practical limit to the depth of the mould which can be used in the manufacture of units from a chemically expanded composition of the type with which this application is concerned. I have discovered that the addition of a very small proportion of certain water soluble compounds of high molecular weight to the slurry greatly increases the stability of the cellular structure in this respect and permits the incorporation of a higher percentage of coarse materials while at the same time allowing the use of moulds considerably deeper than was hitherto possible under these circumstances.

In particular two water soluble cellulose compounds known respectively as ethylmethyl cellulose and sodium carboxymethyl cellulose are very valuable. Using an addition of a small quantity of a 5% solution of one of these compounds together with a suitable wetting agent both the size and regularity of the pore structure can be controlled. In general the higher the proportion of the soluble cellulose compound added the finer will be the pore structure.

The precise mechanism by which these agents act is not known. Two properties which they possess appear to be of prime importance however.

(1) They exhibit the tendency to concentrate as an absorbed layer at an interface.

(2) Their solutions are characterized by exhibiting a very high viscosity even at very low concentrations.

It is tentatively assumed that the stabilisation observed is primarily dependent upon the result of the combination of these two properties. That is to say there is produced a concentration of the agent in the wall of a bubble or cell as soon as it is formed which greatly increases the interfacial viscosity and stiffens and strengthens the system. It would not appear to be irrelevant in this connection that the compounds herein described as being most successful stabilizers are characterised by the fact that they possess polar groups distributed along the length of the molecule, so that one would expect the absorbed molecules to lie more or less parallel to the interface instead of at right angles to it as is the case with the common surface active materials of the hydrocarbon sulphonate type.

If this is the case one can postulate that the presence of a number of these long molecules lying more or less in the surface could behave to some extent as a reinforcement to the fabric of the bubble or cell in a manner not possible with the more simply dipolar surface active compounds which become orientated perpendicular to the interface.

It is to be noted that there exist substances of similar character to the agents named, which are also capable of exerting a stabilizing action on a cellular mix in a like manner and the use of any such agent for this purpose as described herein is included within the invention. For

this reason it is now proposed to define the nature of these compounds.

For the purposes of this invention a cell stabilising agent is defined as a water soluble organic compound of high molecular weight which is surface active and which forms aqueous solutions (true or colloidal) characterised by their abnormally high viscosity at low concentrations of the solute or dispersed phase. Structurally these compounds are generally distinguished by the possession of a number of polar or lyophilic groups distributed along the length of the main molecular axis.

As examples the two soluble cellulose ethers referred to above may be cited.

*Example (A).—Ethylmethyl cellulose*

A mixed ethyl methyl ether of cellulose having generally a degree of substitution in the range of 0.4 to 1.5 hydroxyl groups per glucose unit when produced commercially.

*Example (B).—Sodium carboxymethyl cellulose*

The sodium salt of a carboxymethyl acid of cellulose having generally a degree of substitution in the range of 0.45 to 0.75 hydroxyl group per glucose unit when produced commercially.

Not all wetting agents are equally suitable for use with these stabilisers. I have found that wetting agents of the type which possess hydrophilic groups of the non-dissociating type to be satisfactory in general. In particular a proprietary product known as "Lissapol N" which is described in the literature as being the product of condensing ethylene oxide with a substituted phenol or fatty alcohol has proved to be quite satisfactory and is used as a convenient standard in the examples of suitable compositions which follow.

In my experiments I have used a finely divided type of aluminium powder as the aerating agent, together with a small quantity of caustic soda solution. I have found that six factors are of prime importance in order to ensure a constant degree of aeration and hence a constant density and strength.

- (1) The fineness of the aluminium powder.
- (2) The quantity of the alkali used.

(3) The temperature of the mix.

(4) The consistency of the mix.

(5) The timing of the mixing cycle and particularly the length of time elapsing between the addition of the aerating agents and the discharging of the mix into the mould from the mixer.

(6) The nature and proportion of the stabilising agents used.

Factors (1) and (2) are inter-related in as much as the finer the state of division of the aluminium powder the less is the quantity of alkali required. The quantity of alkali required must be determined by experiment for each type of aluminium powder. It should be sufficient to ensure that the total expansion required takes place in from 10-20 minutes according to the density aimed at.

Aluminium powder is manufactured in a number of grades of fineness. For this purpose it should be at least as fine as that normally supplied for aluminium paint manufacture sometimes known as "varnish grade" and preferably finer. It should also have as low a grease content as possible.

The temperature of the mix is obviously of importance in affecting the rate of evolution of the gas, while it also influences the rate of setting.

I have found it advantageous to use a mix temperature of approximately 40° C. Usually this requires that the gauging water be added at a temperature of 60 to 70° C.

The consistency of the mix has a considerable effect upon the structure and strength of the product.

The ideal consistency is that of a rich creamy slurry, easily pourable, but not wet enough to bleed. The consistency is of course largely determined by the water content. Too little water results in uneven expansion and the formation of large irregular cavities during the pouring. Too much lowers the strength and increases the absorption of the product while also giving rise to a tendency for the mix to slump in the mould. One of the secondary benefits derived from the use of the stabilising agents referred to is that the actual water content is rendered less critical in this respect. Owing to variations in the natural moisture contents of the materials and also the free carbon content of the pulverised fuel ash it has been found impracticable to control the consistency accurately by gauging the water added to the mix. In practice it has proved more satisfactory to add the water until the required consistency is attained as judged by eye or recorded by a suitable instrument.

With regard to the timing of the mixing cycle this, of course, depends upon the size of the mix and the type of mixer. A few general directions may be given, however, and these together with a specific example should serve to demonstrate the important points. I have found that contrary to general practice, it is not advisable to add the aluminium powder with the dry ingredients at the beginning of mixing period. If this is done I have found that reaction with the alkali derived from the cement, and in some cases from the pulverised fuel ash, occurs during the whole of the mixing period. Not only is this wasteful of aluminium powder but also, owing to variations in the free alkali content of the cement and pulverised fuel ash, it leads to variations in the expansion produced. I have found it most advantageous to add the aluminium powder together with the soluble cellulose compound and a suitable wetting agent between 60 and 90 seconds before pouring the mix while the alkali should be added from 30 to 60 seconds before pouring as a 30% solution of caustic soda.

As an example, I give below the mixing schedule for a mix of 10-15 cu. ft. mixed in an open pan mixer for material intended to have a density of approximately 50 lbs./cu. ft.

| Time in Seconds | Schedule                                                                |
|-----------------|-------------------------------------------------------------------------|
| 0.....          | Discharge dry ingredients from hopper.                                  |
| 20-30.....      | Commence addition of water.                                             |
| 130-150.....    | Cease addition of water.                                                |
| 160-180.....    | Add aluminium powder in suspension with stabilising and wetting agents. |
| 190-210.....    | Add requisite quantity of 30% caustic soda solution.                    |
| 250-270.....    | Discharge from mixer.                                                   |

With regard to the quantity of stabilising agent used, fairly wide limits can be set but the use of too high a proportion results in the inhibition of the aeration of the mix to some extent so that the final product is denser than desired. Suitable quantities chosen in relation to the desired pore size, coarseness of sand and so on are determined by experiment. It is important to note that different samples of very similar chemical composition may vary in their ability to

stabilise the mix. It appears that standardisation by the criterion of the viscosity of a dilute (say 1% of solution) of the agent is possible. Alternatively it is not difficult to make slight alterations to the proportions to adjust for variations from batch to batch in the activity of the agent as manufactured.

Having discussed the general nature of the present invention it is now proposed to specify in greater detail the range of compositions and processes covered with several examples.

The present invention has for its object an improved composition and a method of manufacture thereof into a light-weight cellular concrete composition in which the known pozzolanic properties of pulverised fuel ash are utilised, the necessity for grinding the aggregate is eliminated and the time of curing of the concrete is greatly reduced, while the product is characterised by its high strength, durability, low absorption and relatively small changes in dimension on wetting and drying and also its uniformity of structure.

The improved composition consists of a mixture of Portland cement, pulverised fuel ash or fly ash, a suitably graded siliceous sand and a small quantity of very finely divided aluminium powder together with a small proportion of a solution containing a suitable water soluble stabilising compound and a suitable wetting agent, a solution of caustic soda and water. The improved method of manufacture thereof is concerned with the procedure to be adopted in the mixing of the various ingredients, the pouring of the mixture into moulds and the curing of the composition.

The following describes in detail the preparation and manufacture of a lightweight composition having a density of about 55 lbs./cu. ft. The description relates to a mix of approximately 15 cu. ft. of expanded concrete composition mixed in a revolving pan mixer.

#### Example I

The proportions given in the table are such as to produce approximately 15 cu. ft. of the expanded material.

|    | Ingredients                                           | Proportions                                                            |
|----|-------------------------------------------------------|------------------------------------------------------------------------|
| 50 | Portland Cement.....                                  | 224 lbs.                                                               |
|    | Pulverised Fuel Ash.....                              | 268 lbs. (dry weight).                                                 |
|    | Sand 1.....                                           | 180 lbs. (dry weight).                                                 |
|    | Aluminium Powder.....                                 | 9 ozs.                                                                 |
|    | 30% Caustic Soda Solution.....                        | 250-700 mls. according to reactivity of aluminium powder.              |
| 55 | 5% Solution of Sodium Carboxymethyl Cellulose.        | 100-200 mls. according to size of pore desired and activity of sample. |
|    | 10% Solution of Non-ionic Wetting Agent "Lissapol N." | 350 mls.                                                               |

#### 60 1 Grading of sand:

|    | B. S. Sieve No. | Percent Passing |
|----|-----------------|-----------------|
| 65 | 25.....         | 100             |
|    | 52.....         | 75              |
|    | 100.....        | 0               |

The Portland cement, pulverised fuel ash and sand are mixed in the dry state for about 30 seconds. The water is then run in at about 65° C., mixing meanwhile until a homogeneous creamy slurry is obtained. This will take approximately another 100-120 seconds. The aluminium powder is then added as a suspension in a mixture of the wetting agent and the sta-

biliser. Mixing is continued until the aluminium powder is completely dispersed in the mix (about 30 seconds. The measured volume of 30% caustic soda solution is now added and mixing continued for another 60 seconds). By the end of this time if the concentration of alkali has been correctly adjusted the evolution of gas will be proceeding vigorously within the mix. The mix is then ready for pouring. It is poured into an oiled mould which has preferably been preheated to the temperature of the mix. Alternatively the sides of the mould may be made of wood or some other material which is a poor conductor of heat. The quantity of slurry poured into the mould is adjusted so that when the rising is complete there is a slight excess of material over the top of the mould.

The mould and the contents are allowed to stand in a humid atmosphere at room temperature for 3 hours and the excess material is cut off. The sides of the mould can then be removed and the material is ready for cutting into the required sections. Curing may then be commenced, either in moist air, low pressure steam or high pressure steam. The mix described above is designed to be cured in saturated steam at a maximum pressure of 160 lbs./sq. in.

At this pressure a suitable curing cycle has been found to be 3 hours for development of pressure, 7 hours at full pressure and 2 hours depression to atmospheric pressure. With these conditions of curing the following strengths will normally be obtained.

|                          | Lbs./sq. in. |
|--------------------------|--------------|
| Compressive strength wet | 700-800      |
| Compressive strength dry | 950-1050     |
| Modulus of rupture dry   | 330-350      |

This represents a great improvement on the time necessary with conventional Portland cement: sand mix of the same density in order to achieve an equivalent strength.

Having described in detail the composition and method of manufacture of a light-weight material of approximately 55 lbs./cu. ft., I will now give examples of compositions for the manufacture of light-weight materials of various densities for different purposes and suited to various methods of curing.

#### Example II

Light-weight material of approximate density 75 lbs./cu. ft. produced with low pressure steam or moist air curing and suitable for manufacture into internal partition blocks. Strength approximately 600-800 lbs./sq. in. according to method of curing.

| Ingredients                                          | Proportions                     |
|------------------------------------------------------|---------------------------------|
| Portland Cement                                      | 1 part.                         |
| Pulverised Fuel Ash                                  | 1.2 parts.                      |
| Sand                                                 | 2.8 parts.                      |
| Aluminium Powder                                     | 0.0015 part.                    |
| 30% Caustic Soda Solution                            | 1.5-3.5 mls. per lb. of cement. |
| 5% Solution of Sodium Carboxymethyl Cellulose        | 0.5-1.0 mls. per lb. of cement. |
| 10% Solution of Non-ionic Wetting Agent "Lissapol N" | 2.0 mls. per lb. of cement.     |

#### Example III

Light-weight material of approximate density 65 lbs./cu. ft. produced with low pressure or high pressure steam curing. Strength 600-900 lbs./sq. in. according to method of curing.

|    | Ingredients                                          | Proportions                     |
|----|------------------------------------------------------|---------------------------------|
| 5  | Portland Cement                                      | 1 part.                         |
|    | Pulverised Fuel Ash                                  | 1.2 parts.                      |
|    | Sand                                                 | 1.6 parts.                      |
|    | Aluminium Powder                                     | 0.002 part.                     |
|    | 30% Caustic Soda                                     | 1.2-3.2 mls. per lb. of cement. |
| 10 | 5% Solution of Sodium Carboxymethyl Cellulose        | 0.3-0.8 mls. per lb. of cement. |
|    | 10% Solution of Non-ionic Wetting Agent "Lissapol N" | 1.5 mls. per lb. of cement.     |

#### Example IV

Light-weight material of approximate density 45 lbs./cu. ft. suitable for use where a structural material of high insulation value and low shrinkage is required. Curing should be in high pressure steam at 160 lbs./sq. in. to ensure minimum changes in dimensions on wetting and drying.

|    | Ingredients                                          | Proportions                     |
|----|------------------------------------------------------|---------------------------------|
| 20 | Portland Cement                                      | 1 part.                         |
|    | Pulverised Fuel Ash                                  | 1.2 parts.                      |
|    | Sand                                                 | 0.8 part.                       |
|    | Aluminium Powder                                     | 0.030 part.                     |
|    | 30% Caustic Soda Solution                            | 1.2-3.5 mls. per lb. of cement. |
|    | 5% Solution of Sodium Carboxymethyl Cellulose        | 0.3-0.5 mls. per lb. of cement. |
|    | 10% Solution of Non-ionic Wetting Agent "Lissapol N" | 1.5 mls. per lb. of cement.     |

The above examples serve to illustrate the general range of compositions included in this invention, but of course the examples given must not be held to limit the invention as there is a very large number of suitable combinations of the basic ingredients which will provide compositions for manufacture into materials of various densities, strengths, thermal conductivities and shrinkage characteristics and suited to a variety of curing procedures. The choice of a particular composition for a given purpose is governed not only by technical considerations but also by the economic factors involved, and it should be particularly noted that one considerable advantage offered by the successful utilisation of a waste material such as pulverised fuel ash in the production of a high quality light-weight material as herein described lies in the reduction in cost of manufacture effected.

In fact it is true to say that using the compositions and methods specified it is possible to manufacture a material of improved qualities at a cost which is lower than that for conventional light-weight Portland cement:sand or Portland cement:pozzolana:sand mixes whether the pozzolana be either a natural trass or other material specially ground or an artificial product specially prepared by heating and grinding some natural siliceous material.

As an approximate range of the useful and economic compositions the following proportions may be given:

Portland cement, 1 part  
Pulverised fuel ash, 0.3-1.5 parts  
65 Sand, 0.5-4.7 parts  
Powdered aluminium, .001-0.5 part  
1.2 to 3.5 mls. per pound of cement of a 30% caustic soda solution

70 with a very small proportion of sodium carboxymethyl cellulose or of ethyl methyl cellulose and of a non-ionic wetting agent and water.

I claim:

1. Method of producing lightweight concrete consisting in mixing about 1 part of each by

weight of Portland cement and ash from the combustion of pulverised bituminous fuel in furnaces and recovered from the combustion gases by separators with 0.5 to 4.7 parts of sand, adding to the mixture water at a temperature of about 60° to 70° C. in sufficient quantity to form and forming therewith a creamy slurry, adding aluminum powder to the slurry as a dispersion in a solution containing about 0.3 to 1 ml. per pound of cement of a 5% solution of a water soluble stabilising agent of high molecular weight which is surface active and forms an aqueous solution of high viscosity selected from the group consisting of sodium carboxy methyl cellulose and ethyl methyl cellulose and about 1.5 to 2 mls. per pound of cement of a 10% solution of a wetting agent possessing hydrophilic groups of the non-dissociating type, mixing the dispersion with the slurry to produce a thorough dispersion of the aluminum powder, and then adding alkali shortly before discharging the mixture into a mould.

2. Method of producing lightweight concrete consisting in mixing about 1 part each by weight of Portland cement and ash from the combustion of pulverised bituminous fuel in furnaces and recovered from the combustion gases by separators with 0.5 to 4.7 parts of sand, adding to the mixture water at a temperature of about 60° to 70° C. in sufficient quantity to form and forming therewith a creamy slurry, adding aluminum powder to the slurry as a dispersion in a solution containing about 0.3 to 1 ml. per pound of cement

of a 5% solution of a water soluble stabilising agent of high molecular weight which is surface active and forms an aqueous solution of high viscosity selected from the group consisting of sodium carboxy methyl cellulose and ethyl methyl cellulose and about 1.5 to 2 mls. per pound of cement of a 10% solution of a wetting agent possessing hydrophilic groups of the non-dissociating type, mixing the dispersion with the slurry to produce a thorough dispersion of the aluminum powder, adding alkali shortly before discharging the mixture into a mould, allowing the mixture in its mould to stand in a humid atmosphere at room temperature for a number of hours and then curing the mix by means of saturated steam.

PETER EDWARD STARNES.

References Cited in the file of this patent

UNITED STATES PATENTS

| Number    | Name     | Date          |
|-----------|----------|---------------|
| 1,954,117 | Caldwell | Apr. 10, 1934 |
| 2,205,735 | Scherer  | June 25, 1940 |
| 2,432,971 | Ruthman  | Dec. 16, 1947 |
| 2,476,306 | King     | July 19, 1949 |
| 2,534,915 | King     | Dec. 19, 1950 |
| 2,560,871 | Johnson  | July 17, 1951 |

FOREIGN PATENTS

| Number  | Country       | Date         |
|---------|---------------|--------------|
| 243,308 | Great Britain | Dec. 9, 1926 |
| 480,681 | Great Britain | of 1938      |